

## UNITED STATES PATENT OFFICE.

NARAINA DAS CHOPRA AND FREDERICK JOHN BULLEN, OF LONDON, ENGLAND.

## HEAT TREATMENT OF STEEL.

No Drawing. Application filed March 18, 1927, Serial No. 176,585, and in Great Britain April 1, 1926.

This invention relates to heat treatment of steel and has particular reference to heat treatment of alloy steels such, for instance, as tool steels:

5 Steel and steel articles as at present manufactured are frequently defective by reason of a nonuniform distribution of carbon throughout the mass, involving an outer zone of decarburized steel, an inner central zone 10 of a pearlitic nature and an intermediate zone of high-carbon steel. This zonic heterogeneity of structure is generally accompanied by a state of internal instability and has been found, in the case of rolled steel members, 15 such as rails, to be mainly responsible for the commonly experienced disadvantages of corrugating and excessive wear and tear in use. A further disadvantage frequently associated with the presence of the aforesaid 20 zoning of structure is the tendency to distortion of the steel member due to the existence of internal stresses and strains.

The defects referred to above may take place during any post-production heat treatment of steel. For example, in the case of 25 an ingot, billet or the like, the defect may occur during heat treatment in the soaking pit or in the re-heating furnace if the steel be subjected to a process of reheating at any 30 time. Indeed, under the conditions now prevailing in the art, practically any process of heat treatment to which steel or a steel article is subjected will result in the aforesaid uneven 35 distribution of carbon and consequent zonic heterogeneity of structure with its accompanying ill effects upon the performance of the steel in use.

We have discovered that if the furnace atmosphere surrounding the steel during the 40 heat-treatment thereof be one which has been rendered innocuous towards the steel as regards its oxidizing and decarburizing capacity by treatment with both an alkaline earth oxide such as lime and a substantially non- 45 carburizing carbon-carrying material as hereinafter defined, the steel will not become decarburized by the heat-treatment and the zonic non-uniform distribution of carbon throughout the mass will not occur, or if these defects should occur, it would be only to a much reduced degree as compared with treatment in a normal heating atmosphere,

that is to say, in an unmodified atmosphere such as would obtain without the use of the two reagents aforesaid, for example, in the case of furnace-treatment, such as would ordinarily obtain in a soaking-pit, reheating furnace or the like.

In the preceding paragraph reference has been made to "a substantially non-carburizing carbon-carrying material as hereinafter defined." We mean by this, a material consisting of a small proportion (e. g. about 10% or less) of free carbon in association with a sufficiency of inert and substantially incombustible matter, to render the mixture substantially non-carburizing towards the steel under the conditions of the heat-treatment thereof in which it is employed. Materials answering to this description, and which have been 70 found to give satisfactory results, and which, moreover, can be specially recommended for reasons of economy, in that they are not costly materials, are boiler-ash and producer-ash and carburizing mixtures which latter have been used to such an extent as to be rendered more or less unsuitable for further use in carburizing, and which, for brevity, will be referred to herein, as "exhausted carburizing mixtures."

We have found that if, in the case, for example, of heat treatment of a steel ingot in a soaking pit, the heat treatment be effected in the presence of a mixture of two reagents aforesaid,—that is to say, for example, a 85 mixture of lime and boiler-ash, an appropriate quantity of the mixture being added to the furnace and maintained therein during the treatment, the ingot will not become decarburized and rendered non-uniform in its 90 structure as regards carbon distribution. Moreover, we have found that under these conditions the ingot, billet or the like, may be left in the soaking pit or other form of furnace practically indefinitely, at any rate 95 for a much longer period than heretofore, without the deleterious effect on the steel of over-heating.

A further disadvantage, frequently, if not invariably, associated with heat treatment of 100 steel as at present conducted, is the considerable formation of scale on the surface of the steel or steel article, due, of course, to oxidation by the surrounding atmosphere during

the heat treatment. We have found that this disadvantage, as well as those hereinbefore referred to, is very materially, if not entirely, overcome and that the steel or steel article 5 heat-treated under the conditions characteristic of this invention will be substantially free from oxidation.

We have referred above to heat treatment of steel in a soaking pit. The novel effect, 10 however, is obtainable in any process of heat treatment and is not confined to heat treatment within a heating chamber such as a furnace. For instance, it is possible in the case of the manufacture of steel rails where ordinarily the finished rail is transferred from the rolling mills to the hot banks after the last rolling operation and there allowed to cool, to secure complete homogeneity of structure and avoidance of the decarburization and oxidation, by burying the hot rail in a mixture of 15 the two modifying reagents referred to above.

As will be readily appreciated from the foregoing, the term "normal atmosphere" as used above denotes the atmosphere which ordinarily surrounds a steel member in any of 25 the normal processes in the art of heat treatment of steel by direct contact with hot furnace gases, and is not limited to the furnace atmosphere of a soaking pit, re-heating furnace and the like.

Furthermore, it is immaterial whether the heat treatment be one which involves a raising of temperature of the steel or a lowering of temperature.

30 It has been found that for the best results it is important that the alkaline earth oxide should be employed in a certain definite proportion in relation to the carbon-carrying material. Thus, it has been found that the 35 relative amounts of the two reagents should be such that the quantity of oxide employed is equivalent to from 10% to 50% by weight of the combined quantities of oxide and carbon-carrying material, and the carbon-con- 40 tent of the carbon-carrying material should be such that the quantity of free carbon present is equivalent to from 4% to 20% by weight of the aforesaid combined quantities.

We have also found in our investigations 45 that the novel effects characteristic of the invention can be enhanced by conducting the heat treatment of the steel in a modified furnace atmosphere as aforesaid and in the presence of material, such, for example, as 50 scrap steel plates, (say, scrap steel known in the art as tin plate) steel wire spools or spirals, scrap steel of any description, for example, steel turnings, filings, mill cuttings, etc. which is readily oxidizable, is unreactive 55 deleteriously upon the steel under heat treatment at the temperature employed, and is of such form as will enable it to present to the surrounding atmosphere an area of oxidizable surface which is large relatively to the 60 mass of the material. The degree of decar- 65

burization and scale formation appears to be approximately proportional to the surface area of metal exposed. Consequently, a false, increase of area, such as would be provided by the presence of material of above 70 type, will reduce the degree of possible oxidization of the steel per unit of area and correspondingly also the extent of decarburization.

According to a further feature of the invention, therefore, steel is heat treated in a modified atmosphere as aforesaid in the presence of material, such, for example, as that referred to above, which is readily oxidizable, is unreactive deleteriously upon the steel 80 under heat treatment at the temperature employed, and is of such form as will enable it to present to the surrounding atmosphere an area of oxidizable surface which is large relatively to the mass of the said material.

85 It is to be appreciated that the process of the present invention is a process which depends upon certain specific chemical interactions as between the furnace gases and the constituents of the steel of the member under 90 treatment. It is, therefore, to be distinguished from processes of simple annealing, normalizing, refining and the like, which, in general, are processes involving only transformations of a physical nature. The following will, perhaps, make this clear.

95 If a mass of steel is heated it behaves more or less like an open sponge, and the furnace gases by which the steel is heated tend to penetrate into the interior of the mass and either rob the steel of a proportion of its carbon by attacking the iron carbide components of the steel, or deposit carbon which combines with the ferrite present in the steel. The net result of this action of the furnace gases upon 100 the steel depends upon the amount of free carbon or free oxygen present in the gases and varies with a definite effect according to 105 which of the two predominates. It has been determined, however, that the degree and intensity of action of the gases upon the steel is dependent to a considerable extent upon the presence of certain hydrocarbon constituents 110 of the gases. It has been found as the result 115 of our investigations that these hydrocarbon constituents act as accelerating agents or catalysts in relation to the steel-attacking components of the furnace gases. These investigations lie behind the present invention, and we have found that by the special means hereinbefore stated, both the accelerating action of the hydrocarbon constituents of the gas, and also the action of the steel-attacking constituents, can be prevented, or at any rate 120 neutralized, with the result that a rail or other steel-member may be produced which is free from the oxidation decarburizing and kindred defects hereinbefore mentioned.

125 The amounts to be used of steel shavings, scrap steel plate, steel wire spools, spirals etc.

and lime or other alkaline earth oxide and exhausted carburizing mixture or other carboniferous material employed will be found to depend upon circumstances in any given case. Thus, the amounts will be found to vary with the type of steel under treatment, that is to say, with the analysis of the steel, particularly in relation to its liability to oxidation, the weight of steel in any one furnace, the area of steel exposed to the gases in relation to the volume of gases supplied to the furnace, the design of the furnace, and lastly, the actual chemical composition of the furnace gases themselves. As will be appreciated, the aforesaid are all variable factors and as they all have a bearing upon the actual amounts of scrap steel or the like to be employed in any given case, it will be at once understood that it is practically impossible to stipulate a rule governing the amounts of the materials to be employed. In actual practice it is a simple matter for a workman operating the process to determine by judgment or trial and adjustment the appropriate amounts to be used. Moreover, there are certain indications in the actual furnace practice of the process, such as the appearance of the flame from the furnace and the general appearance of the furnace, which would guide the operator in determining whether sufficient of the modifying reagents is being used. The use of the modifying reagents involves the presence in the furnace of a reducing atmosphere and, generally speaking, therefore, the appearance of the furnace would be a ready guide as to whether the quantity in use of the modifying reagents is sufficient.

If an exhausted carburizing mixture is used, a suitable mixture is one which, prior to its use as a carburizing agent, was composed of three parts of powdered beech charcoal, two parts of powdered horn charcoal and two parts of powdered animal charcoal, and which has been used to such an extent as to render it unsuitable for further use in carburizing.

The special heat treatment constituting the present invention has been found to be utilizable, not only for the purpose of avoiding the structural defects hereinbefore referred to during the manufacture of a steel article, but also for the removal of such defects after manufacture. It has been found that if steel or a steel article, defective as aforesaid by reason of decarburization and zonic heterogeneity of structure, be heat treated preferably through a range of temperatures embracing the change-points of the steel in an atmosphere modified according to the present invention, the defects will be materially, if not entirely, removed, the structure being rendered uniform throughout as regards carbon distribution, and the carbon content of the steel being restored to what it would have

been had not decarburization taken place in the previous heat treatment to which the steel had been subjected.

The invention is capable of wide application and is moreover susceptible to extensive variation in the matter of proportions, temperatures, and other conditions of its use.

The following is a detailed example illustrating the invention in its application to the manufacture of steel billets for various purposes.

In normal works practice as hitherto carried out, the steel ingot has been stripped and heated in furnace pits prior to rolling. The time of heating in the pits has varied from 6 to 10 hours, according to works exigencies. At the end of the period the ingot has been passed through the blooming and rolling mills until the required section had been obtained, and thereafter to the hot shears, where bottom and top crops were taken, and finally to the stores.

In applying the process of this invention a mixture was prepared consisting of one part by weight of lime and eight parts by weight of boiler ash carrying about 10% of combustible carbon. This mixture was left to dry for two days before application. No particular efforts was made to reduce this mixture to any definite size mesh.

The mixture was spread to a depth of 6" on the floor of the furnace before firing the latter. On top of the bed so formed steel turnings were spread to the depth of another 2". On charging each ingot four shovelsful of the mixture were thrown on to the ingots, together with two shovelsful of the turnings. In addition to this, material was thrown on to the lip of the gas inlet ports so that the incoming gases had to pass through the small heap of the material left at the end of the ports. After heating under these conditions the ingot was treated in the normal way, viz passed through the blooming and rolling mills, cropped at each end, and passed to stores.

The approximate loss of weight between the metal charged in the pits and the finished billets, including crops, was before the application of the process in the region of 4% by weight. The following are representative figures of ingots taken from a batch treated under this invention:—

#### Medium carbon steel.

| State of<br>ingot<br>when<br>charged | Time<br>(in<br>hours)<br>in the<br>pits. | Weight<br>charged<br>(kgs.). | Weight after rolling. |        |        | Losses.    |                 | Re-<br>marks.      |
|--------------------------------------|------------------------------------------|------------------------------|-----------------------|--------|--------|------------|-----------------|--------------------|
|                                      |                                          |                              | Bil-<br>lets.         | Crops. | Total. | In<br>kgs. | In per<br>cent. |                    |
| Cold...                              | 6.30                                     | 1821                         | 1615                  | 195    | 1810   | 11         | 0.59            |                    |
| Hot...                               | 10.20                                    | 1417                         | 1312                  | 97     | 1409   | 8          | 0.565           |                    |
| Hot...                               | 10.0                                     | 1400                         | 1310                  | 90     | 1400   | 0.0        | 0.0             | Billets<br>150 m/m |

In addition, steel so treated showed greater

freedom from ingot defects, and in general was of better quality.

In another application of the invention a batch of steel files were treated to harden the 5 steel.

First, one batch of files were hardened by the ordinary treatment in a gas-fired muffle furnace. The files on completion of the treatment were heavily scaled and were characterized moreover by local zones of decarburization.

A second batch of files were then taken and heat-treated in the same gas-fired muffle under exactly the same conditions but in the 15 presence of a mixture of 2 parts of lime and 3 parts of exhausted carburizer containing about 15% of free carbon when introduced into the furnace, this mixture being disposed in the muffle in a bed on the bottom thereof 20 approximately six inches deep and the files being placed upon this bed. At the conclusion of the hardening process the files were removed and found to be properly hardened, free from scale and free from soft spots, that 25 is to say, areas of decarburization.

Similarly, tool steel was heat-treated in an electric furnace for the purpose of hardening the steel both with and without modification of the furnace atmosphere according to the 30 present invention. Without modification, that is to say, heat treatment of the tool steel in the ordinary way, resulted in considerable oxidation and local decarburization of the steel. The same treatment repeated on another batch 35 of the same steel in the presence of a mixture of lime and boiler ash, the latter component carrying about 15.6% of combustible carbon, and the two components being present in approximately the relative proportions of 40:60, 40 resulted in proper hardening of the steel with complete avoidance of scale formation and decarburization of the steel. The aforesaid mixture of lime and boiler ash was disposed as a bed of approximately 4 inches in depth upon 45 the bottom of the furnace and after the steel had been placed in the furnace a further charge of the mixture was introduced loosely around the steel in the space between the steel and the walls of the furnace. In addition to 50 the mixture of lime and boiler ash there was present in the furnace a quantity of steel turnings. These were intermixed with the lime and boiler ash in the bed of the latter upon the floor of the furnace and the space around 55 the sides and above the top of the steel under treatment was occupied by steel spirals suspended from the sides and the top of the furnace. The spirals were suspended at intervals of approximately 4 inches across the under- 60 side of the top of the furnace. Further steel scrap was thrown into the furnace at intervals during the treatment.

The invention has been found to be particularly successful in the heat treatment of ar-

mour plate, for example, for purposes of 65 hardening and toughening the same.

As stated before, the invention is applicable to heat treatment in any type of furnace whether electric, gas-fired or furnaces of the open-hearth type.

We claim:—

1. In processes of heat treatment of steel wherein the steel is heated by direct contact with furnace gases, effecting the treatment in and by hot furnace gases which have been 70 rendered substantially innocuous towards the steel as regards their oxidizing and decarburizing capacity by treatment with a mixture of an alkaline earth oxide and a carbon-carrying material consisting of carbon in association with a sufficiency of ash to render the material substantially non-carburizing towards the steel.

2. In processes of heat treatment of steel wherein the steel is heated by direct contact with furnace gases, effecting the treatment in and by hot furnace gases which have been 75 rendered substantially innocuous towards the steel as regards their oxidizing and decarburizing capacity by treatment with both an alkaline earth oxide and a carbon-carrying ash which has been produced by the partial combustion of a carbonaceous material and which contains an insufficiency of residual 80 combustible carbon to render the ash materially carburizing towards the steel.

3. In processes of heat treatment of steel wherein the steel is heated by direct contact with furnace gases, effecting the treatment in and by hot furnace gases which have been 85 rendered substantially innocuous towards the steel as regards their oxidizing and decarburizing capacity by treatment with both an alkaline earth oxide and a substantially non- 90 carburizing carbon-carrying material as herein defined, the quantity of oxide employed being equivalent to from 10% to 50% by weight of the combined quantities of the oxide and the carbon-carrying material and the carbon content of the carbon-carrying material being such that the quantity of free 95 carbon present is equivalent to from 4% to 20% by weight of the aforesaid combined quantities.

4. In processes of heat treatment of steel wherein the steel is heated by direct contact with furnace gases, effecting the treatment in and by hot furnace gases which have been 100 rendered substantially innocuous towards the steel as regards their oxidizing and decarburizing capacity by treatment with both lime and a carbon-carrying ash which has been produced by the partial combustion of carbonaceous material, the quantity of lime employed being equivalent to from 10% to 50% 105 by weight of the combined quantities of the lime and the ash and the carbon content of the ash being such that the quantity of free 110

120

125

carbon present is equivalent to from 4% to 20% by weight of the aforesaid combined quantities.

5. In processes of heat treatment of steel wherein the steel is heated by direct contact with furnace gases, effecting the treatment in and by hot furnace gases which have been rendered substantially innocuous towards the steel as regards their oxidizing and decarburizing capacity by treatment with both an alkaline earth oxide and a substantially non-carburizing carbon-carrying material as herein defined and with a material which is readily oxidizable, is infusible and unreactive 10 upon the steel under heat treatment at the temperature employed and is of such form as will enable it to present to the surrounding atmosphere an area of oxidizable surface which is large relatively to the mass of the 20 infusible material.

6. In processes of heat treatment of steel wherein the steel is heated by direct contact with furnace gases, effecting the treatment in and by hot furnace gases which have been rendered substantially innocuous towards the steel as regards their oxidizing and decarburizing capacity by contact with a false area of oxidizable surface provided by a mass of scrap steel of extended superficial area, and 25 by treatment with both lime and a carbon-carrying ash which has been produced by the partial combustion of a carbonaceous material, the quantity of lime employed being equivalent to from 10% to 50% by weight of 30 the combined quantities of the lime and ash and the carbon-content of the ash being such that the quantity of free carbon present is equivalent to from 4% to 20% by weight of the aforesaid combined quantities.

40 7. The process of rendering innocuous the atmosphere in which an iron alloy is being heated, which comprises subjecting the atmosphere to the action of material which renders it substantially innocuous toward the 45 alloy as regards its oxidizing and decarburizing and rebarburizing properties.

8. The process of rendering innocuous the atmosphere in which an iron alloy is being heated, which comprises subjecting the atmosphere to the action of material containing 50 an alkaline earth oxide and a reducing agent.

55 9. The process of rendering innocuous the atmosphere in which an iron alloy is being heated, which comprises subjecting the atmosphere to the action of material containing an alkaline earth oxide and carbon.

60 10. The process of rendering innocuous the atmosphere in which an iron alloy is being heated, which comprises subjecting the atmosphere to the action of material containing an alkaline earth oxide and carbon, the material being substantially non-carburizing toward the alloy.

65 11. The process of rendering innocuous the

atmosphere in which an iron alloy is being heated, which comprises subjecting the atmosphere to the action of an alkaline earth oxide and a carbonaceous material, the quantity of the alkaline earth oxide employed being equivalent to at least 10% by weight of the combined quantities of the oxide and carbonaceous material.

70 12. The process of rendering innocuous the atmosphere in which an iron alloy is being heated, which comprises subjecting the atmosphere to the action of an alkaline earth oxide and a carbonaceous material, the quantity of combustible carbon present in the carbonaceous material being equivalent to at 80 least 4% by weight of the combined quantities of the oxide and the carbonaceous material.

75 13. The process of rendering innocuous the atmosphere in which an iron alloy is being heated, which comprises subjecting the atmosphere to the action of an alkaline earth oxide and a carbonaceous material, the quantity of the alkaline earth oxide being equivalent to from 10 to 50% by weight of the combined quantities of the oxide and the carbonaceous material.

80 90 14. The process of rendering innocuous the atmosphere in which an iron alloy is being heated, which comprises subjecting the atmosphere to the action of an alkaline earth oxide and a carbonaceous material, the carbon content of the carbonaceous material being such that the quantity of combustible carbon present is equivalent to from 4 to 20% by weight of the combined quantities of the oxide and the carbonaceous material.

85 95 100 105 110 115 120 125 130 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 9900 9905 9910 9915 9920 9925 9930 9935 9940 9945 9950 9955 9960 9965 9970 9975 9980 9985 9990 9995 10000 10005 10010 10015 10020 10025 10030 10035 10040 10045 10050 10055 10060 10065 10070 10075 10080 10085 10090 10095 10100 10105 10110 10115 10120 10125 10130 10135 10140 10145 10150 10155 10160 10165 10170 10175 10180 10185 10190 10195 10200 10205 10210 10215 10220 10225 10230 10235 10240 10245 102

line earth oxide and a carbonaceous material, and prolonging the effective life of said mixture by adding a material which is readily oxidizable and unreactive upon the alloy at the temperature employed and which presents a large surface area as compared with that of the alloy, said material also serving to pre-

vent decarburization of the iron alloy in case the carbonaceous material becomes ineffective.

In testimony whereof we have signed our names to this specification.

NARAINA DAS CHOPRA.  
FREDERICK JOHN BULLEN.